

Nov. 18, 1941.

W. WHITEHEAD

2,262,872

METHOD OF PREPARING TEXTILE MATERIALS

Filed June 1, 1938



INVENTOR  
William Whitehead

BY  
*J. Seltzer & Co. Levinson*  
ATTORNEYS

## UNITED STATES PATENT OFFICE

2,262,872

## METHOD OF PREPARING TEXTILE MATERIALS

William Whitehead, Cumberland, Md., assignor to  
Celanese Corporation of America, a corporation  
of Delaware

Application June 1, 1938, Serial No. 211,205

18 Claims. (Cl. 18—54)

This invention relates to the manufacture of yarns, and particularly yarns of cellulose acetate or other organic derivative of cellulose, having the appearance of spun yarn or yarn made from staple fiber, and relates also to fabrics made from such yarns.

This application is a continuation-in-part of my application S. No. 205,990, filed May 4, 1938.

An object of the invention is the economic production of "staplized yarn," i. e. one having the appearance of being composed of short lengths of fiber spun into a yarn and which is formed of continuous filaments which, after the filaments are grouped together to form a yarn, are subjected to an operation to break the continuity of some, but not all, of the filaments associated in the yarn, so that the resulting yarn has a number of broken ends which give it, when twisted, the appearance of a spun yarn. Another object of the invention is to reduce the number of steps formerly necessary to produce such a yarn. A still further object of the invention is the production of a more uniform and stronger staplized yarn which, therefore, may be knitted into circular knit fabrics with less presser marks, holes and other faults. A still further object of the invention is the product of a staplized yarn which knits into a fabric characterized by having softer hand. Other objects of the invention will appear from the following detailed description.

Imitation spun yarn, or staplized yarn, has been made by processes where some filaments of a continuous filament yarn are broken to break the continuity of same. Such a process is described in U. S. Patent No. 2,098,980 to Sowter. Other methods have been employed wherein some of the filaments of the yarn are cut or torn to produce a similar effect. I have now found that a yarn having the appearance of a spun yarn may be produced more economically and at the same time stronger yet capable of being knitted into a softer fabric.

In accordance with my invention, I spin a yarn from a solution of a suitable organic derivative of cellulose in a solvent therefor by extruding the solution through a jet into a drying atmosphere or a precipitating medium, under such conditions that the resulting yarn contains at least two sizes of filaments. One method of accomplishing this is to have two jets in the same cabinet, one jet having fine holes and the other jet having coarser holes both fed by the same pump. Also two separate jets may be employed in the same cabinet, the jets having the same size holes but fed by separate pumps, where the debit of the pumps

will produce different size filaments. The filaments from the two jets are led from the cabinet together and are wound on to the same bobbin. Another method of carrying my invention into effect is to produce one end of fine filament yarn and one end of a coarser filament yarn in adjacent cabinets and draw the same together by a feed roll and then wind them on to the same bobbin. Still another method of producing a yarn in accordance with the instant invention, although this method is less desirable as it requires an additional step, is the plying together of a fine filament yarn and a coarser filament yarn from suitable supply packages. The yarn containing different size filaments and while it contains little or no twist, say under 5 to 10 turns per inch and preferably about 1 or less turn per inch, is subjected to a staplizing action by stretching and breaking the finer denier filaments leaving the coarser filaments unbroken. This yarn may then be further twisted, doubled, etc. and woven, knitted or knotted into a fabric. This yarn may be the sole yarn in the fabric or it may be used in connection with other types of yarn.

This invention aims to produce a staplized yarn of cellulose acetate or other organic derivative of cellulose. Examples of other organic derivatives of cellulose are the cellulose esters such as cellulose formate, cellulose propionate and cellulose butyrate, and the cellulose ethers such as ethyl cellulose, methyl cellulose and benzyl cellulose. It is also applicable to yarns of regenerated or reconstituted cellulose, which yarns are formed by extruding a solution of suitable cellulosic material through a jet to form substantially continuous filaments.

Any number of filaments may be built up into a yarn, say from 20 to 200 or more. These filaments may be of two different sizes or may be of three or more sizes, it being understood that the finer the filament the more readily it is reduced to staple length in the staplizing operation. Any weight and number of yarns may be produced, say from 30 denier to 1,000 denier or more and from 30 to 1,000 filaments or more in number. For instance, yarns in accordance with this invention may be formed from 1,000 denier 104 filaments, 750 denier 150 filaments, 170 denier 40 filaments, 220 denier 40 filaments, 180 denier 60 filaments, 170 denier 60 filaments or any other suitable filament denier and count arrangement. For instance, the yarn to be staplized may be made by spinning one end of 85 denier 25 filament yarn from one jet and of 85 denier 40 filament yarn from another jet in the same cabinet, and

drawing these two yarns together at the feed roll and winding them on to the same bobbin. As there can be little drawing or drafting action during the twisting or formation of the staplized yarn unless stretching of the heavier filaments is resorted to, which stretching is within the scope of this invention, the size of the twisted yarn will be slightly larger than the yarn as it is spun, i. e., as it issues from the spinning device and contains little or no twist.

The yarn containing two or more sizes of filaments as it issues from a spinning device or taken from a package may have the finer filaments broken by leading the same through two sets of nip rollers, the forward set, i. e. the set from which the yarn issues, being driven under slightly greater speed than the rear set. These two sets of nip rollers may be spaced from 1 inch to 10 or more inches apart and the spacing thereof will determine the length of fiber into which the smaller denier or weaker filaments are broken. After the yarn leaves the forward nip rollers it may have twist inserted therein or it may be wound into a package and then twisted upon a separate device. Also, the yarn thus produced may be doubled with a similar yarn, a continuous filament yarn, or a yarn formed of staple fiber. If desired, some drafting of the yarn may be accomplished by subjecting the yarn prior to its entrance into the nip rollers to the softening action of a solvent vapor, steam or other medium which will allow the larger denier or stronger filaments to stretch while the smaller denier or weaker filaments are broken and drafted during the stretching of the larger filaments.

The continuous filament yarns may be staplized by any suitable method. In place of the method described above, which requires stretching of the filaments to the breaking point, it may be staplized, for instance, by abrading rolls with little or no stretching or drafting. In this modification the first pair of rolls which the yarn encounters does not form a true nip. The lower roll of the pair is milled, i. e. has a rough surface and the top roll is comparatively light and bears down on the yarn with only a very light self-load. The second pair of rolls which the yarn encounters forms a definite nip under relatively high load and controls the linear speed of the yarn. The second pair of rolls pulls the yarn forward at a linear speed greater than the peripheral speed of the milled roll of the first pair. Inasmuch as this first pair of rolls is travelling at a surface speed less than that of the yarn and the top roll does not form a positive nip, the yarn slips forward and is broken in places, which are variably spaced, on this pair of abrading rolls. The lower denier filaments break more readily than the coarser filaments.

The yarns prior to or after the operation which breaks the smaller denier or weaker filaments may be subjected to any of the processes now employed to change the physical or chemical nature thereof. For instance, the yarns may be treated and boiled in water to produce a de-lustered yarn; they may have sizes and lubricants applied thereto, they may have dyes and fugitive tints applied thereto, or they may be otherwise modified. The basic yarn may be of high, medium or low luster, the luster being modified, for example, by the incorporation of pigments, by treatment with boiling soap solution or other aqueous liquors or by any other method. Similarly the yarns doubled with the yarns of the present invention may be of normal luster

or the luster may be suitably modified. The association of lustrous and non-lustrous yarns or filaments may take place before or after the breaking of constituent filaments.

- 5 The yarns or mixed yarns of the invention may be woven, knitted or otherwise made up into fabrics consisting solely of said yarns or containing them in admixture with other yarns. For example, the yarns may be introduced into the 10 weft or warp, or both, to produce a woven fabric having the appearance of one constituted wholly of staple fiber yarn or having pattern effects with or without differential luster. The invention is particularly applicable to knitted 15 fabrics of all kinds where the yarns of this invention constitute the sole or principal constituent of the fabric. Knitted fabrics made of yarns produced in accordance with this invention are 20 exceptionally well suited for ladies' underwear fabrics as they have the appearance of being made of staple length fiber and yet they are extremely soft and have high covering power.

As an illustration of this invention, but without being limited thereto, the following examples are given:

#### Example I

A 25% solution of cellulose acetate dissolved in acetone is extruded through suitable spinning jets to produce a yarn. This yarn is formed of 30 one end of an 85 denier 20 filament yarn spun from one jet and an end of 85 denier 40 filament yarn spun from another jet in the same cabinet. These ends are drawn together at the feed roll and wound on to the same bobbin producing a 35 yarn of 170 denier 60 filaments and contains about 1 turn per inch of twist. The yarn is then placed on a staplizing device and passed to the two sets of rollers, the abrading rolls or the first 40 pair of rolls which the yarn encounters being spaced about 5" from the second pair of rolls, which travels at a higher speed than the first set of rolls, in such a manner that the finer filaments are bruised or abraded and thereby broken 45 into 6" lengths, while the coarser filaments remain substantially continuous. This yarn is then given between 5 and 10 turns per inch twist, and a fabric knitted therefrom by a circular knitting operation. The yarn runs exceptionally well in 50 circular knitting machines and the total faults per yard are below 0.08.

#### Example II

Cellulose acetate threads formed by spinning a suitable solution of cellulose acetate through jets is formed from one end of 110 denier 20 filament yarn and one end of 60 denier 20 filament 55 yarn spun in adjacent cabinets and drawn together at the feed roll and wound on to the same bobbin with a twist of about 0.6 turn per inch. This yarn is passed through the staplizing device similar to the yarn of Example I. The yarn is then twisted to from 5 to 10 turns per inch and knitted by circular knitting into a fabric. The yarn runs exceptionally well in circular knitting machines and the fabric produced contains no thin places or slab holes and has substantially no faults.

The above examples are merely illustrative of 70 yarns that may be produced in accordance with this invention. Where three sizes of filaments are employed in building up the same yarn, for instance, all of the smaller denier or weakest filaments will be broken and a part of the medium sized filaments may be broken while the

coarser filaments will be substantially continuous. Although this invention is applicable to yarns having two or more sizes of filaments regardless of how they are formed, I have found it preferable to spin the yarn from one cabinet having at least two jets therein, each jet having different size holes. This arrangement allows for the use of standard jets in the production of yarn without the necessity of reaming out a part of the holes of a standard jet.

One arrangement for carrying out my invention will now be described with reference to the accompanying diagrammatic drawing.

The drawing shows a spinning cell 1 containing two jets 2 and 3 from which bundles of filaments 4 and 5, each bundle containing filaments of a denier different than the other, are extruded in a downward direction and are withdrawn from the cell through an opening 6. The bundles of filaments 4 and 5 are led from opening 6 over 20 a draw roller 7 and through pairs of rollers 8, 8 and 9, 9, each pair of which are operated at different speeds and in such a manner as to break only the filaments of smaller denier. The combined bundles of filaments, now containing staple fibers, are passed through a guide 11 on to a suitable collecting device 12.

It is to be understood that the foregoing detailed description is merely given by way of illustration and that many variations may be made therein without departing from the spirit of my invention.

Having described my invention, what I desire to secure by Letters Patent is:

1. Process for the manufacture of staplized yarn, which comprises producing from a solution of cellulosic material a yarn of substantially continuous filaments of at least two different deniers and, while retaining said filaments in association as a yarn, dividing the filaments of smaller denier into short lengths and leaving the heavier filaments in substantially continuous form.

2. Process for the manufacture of staplized yarn, which comprises producing from a solution of an organic derivative of cellulose material a yarn of substantially continuous filaments of at least two different deniers and, while retaining said filaments in association as a yarn, dividing the filaments of smaller denier into short lengths and leaving the heavier filaments in substantially continuous form.

3. Process for the manufacture of staplized yarn, which comprises producing from a solution of cellulose acetate material a yarn of substantially continuous filaments of at least two different deniers and, while retaining said filaments in association as a yarn, dividing the filaments of smaller denier into short lengths and leaving the heavier filaments in substantially continuous form.

4. Process for the manufacture of staplized yarn, which comprises producing a yarn from a solution of cellulosic materials having substantially continuous filaments of at least two different deniers and subjecting the yarn to a strain whereby the smaller denier filaments are broken and the heavier filaments are left in substantially continuous lengths.

5. Process for the manufacture of staplized yarn, which comprises producing a yarn from a solution of an organic derivative of cellulose material having substantially continuous filaments of at least two different deniers and subjecting the yarn to a strain whereby the smaller denier

filaments are broken and the heavier filaments are left in substantially continuous lengths.

6. Process for the manufacture of staplized yarn, which comprises producing a yarn from a solution of cellulose acetate material having substantially continuous filaments of at least two different deniers and subjecting the yarn to a strain whereby the smaller denier filaments are broken and the heavier filaments are left in substantially continuous lengths.

7. Process for the manufacture of staplized yarn, which comprises producing a yarn from a solution of cellulosic material having substantially continuous filaments of at least two different deniers and subjecting the yarn to a controlled abrading action whereby the smaller denier filaments are broken and the heavier filaments are left in substantially continuous lengths.

8. Process for the manufacture of staplized yarn, which comprises producing a yarn from a solution of an organic derivative of cellulose material having substantially continuous filaments of at least two different deniers and subjecting the yarn to a controlled abrading action whereby the smaller denier filaments are broken and the heavier filaments are left in substantially continuous lengths.

9. Process for the manufacture of staplized yarn, which comprises producing a yarn from a solution of cellulose acetate material having substantially continuous filaments of at least two different deniers and subjecting the yarn to a controlled abrading action whereby the smaller denier filaments are broken and the heavier filaments are left in substantially continuous lengths.

10. Process for the manufacture of staplized yarn, which comprises extruding a solution of cellulosic material through two jets having holes of different sizes and located in the same cabinet, associating the extruded material to form a yarn of substantially continuous filaments of at least two different deniers and, while retaining said filaments in association as a yarn, dividing the filaments of smaller denier into short lengths and leaving the heavier filaments in substantially continuous form.

11. Process for the manufacture of staplized yarn, which comprises extruding a solution of an organic derivative of cellulose material through two jets having holes of different sizes and located in the same cabinet, associating the extruded material to form a yarn of substantially continuous filaments of at least two different deniers and, while retaining said filaments in association as a yarn, dividing the filaments of smaller denier into short lengths and leaving the heavier filaments in substantially continuous form.

12. Process for the manufacture of staplized yarn, which comprises extruding a solution of cellulose acetate material through two jets having holes of different sizes and located in the same cabinet, associating the extruded material to form a yarn of substantially continuous filaments of at least two different deniers and, while retaining said filaments in association as a yarn, dividing the filaments of smaller denier into short lengths and leaving the heavier filaments in substantially continuous form.

13. Process for the manufacture of staplized yarn, which comprises spinning a solution of an organic derivative of cellulose into a yarn of substantially continuous filaments, spinning a second

solution of an organic derivative of cellulose into a second yarn of substantially continuous filaments having a heavier denier than the first yarn, drawing the two yarns together to form a unitary yarn and, while retaining said two yarns together as a unitary yarn, dividing the filaments of smaller denier into short lengths and leaving the heavier filaments in substantially continuous form.

14. Process for the manufacture of staplized yarn, which comprises spinning a solution of cellulose acetate into a yarn of substantially continuous filaments, spinning a second solution of cellulose acetate into a second yarn of substantially continuous filaments having a heavier denier than the first yarn, drawing the two yarns together to form a unitary yarn and, while retaining said two yarns together as a unitary yarn, dividing the filaments of smaller denier into short lengths and leaving the heavier filaments in substantially continuous form.

15. Process for the manufacture of staplized yarn, which comprises spinning a solution of an organic derivative of cellulose into a yarn of substantially continuous filaments, spinning a second solution of an organic derivative of cellulose into a second yarn of substantially continuous filaments having a heavier denier than the first yarn, twisting the two yarns together with a twist of about one turn per inch to form a unitary yarn and, while retaining said two yarns together as a unitary yarn, dividing the filaments of smaller denier into short lengths and leaving the heavier filaments in substantially continuous form.

16. Process for the manufacture of staplized yarn, which comprises spinning a solution of cellulose acetate into a yarn of substantially continuous filaments, spinning a second solution of cellulose acetate into a second yarn of substan-

tially continuous filaments having a heavier denier than the first yarn, twisting the two yarns together with a twist of about one turn per inch to form a unitary yarn and, while retaining said two yarns together as a unitary yarn, dividing the filaments of smaller denier into short lengths and leaving the heavier filaments in substantially continuous form.

17. Process for the manufacture of staplized yarn, which comprises spinning a solution of an organic derivative of cellulose into a yarn of substantially continuous filaments, spinning a second solution of an organic derivative of cellulose into a second yarn of substantially continuous filaments having a heavier denier than the first yarn, twisting the two yarns together with a twist of about one turn per inch to form a unitary yarn and, while retaining said two yarns together as a unitary yarn, dividing the filaments of smaller denier into short lengths and leaving the heavier filaments in substantially continuous form by passing said unitary yarn through the nips of rotary surfaces moving at different rates of speed.

18. Process for the manufacture of staplized yarn, which comprises spinning a solution of cellulose acetate into a yarn of substantially continuous filaments, spinning a second solution of cellulose acetate into a second yarn of substantially continuous filaments having a heavier denier than the first yarn, twisting the two yarns together with a twist of about one turn per inch to form a unitary yarn and, while retaining said two yarns together as a unitary yarn, dividing the filaments of smaller denier into short lengths and leaving the heavier filaments in substantially continuous form by passing said unitary yarn through the nips of rotary surfaces moving at different rates of speed.

40 WILLIAM WHITEHEAD.